

March 18, 1947.

W. W. EITEL ET AL

2,417,458

ELECTRODE

Original Filed July 28, 1943



INVENTORS  
WILLIAM W. EITEL  
JACK A. McCULLOUGH  
BY *Harold E. Say*  
THEIR ATTORNEY

## UNITED STATES PATENT OFFICE

2,417,458

## ELECTRODE

William W. Eitel, Woodside, and Jack A. McCullough, Millbrae, Calif., assignors to Eitel-McCullough, Inc., San Bruno, Calif., a corporation of California

Original application July 28, 1943, Serial No. 496,686. Divided and this application March 20, 1944, Serial No. 527,294

4 Claims. (Cl. 250—177)

1

This is a division of our copending application Serial No. 496,686, filed July 28, 1943.

Our invention relates to electron tubes, and more particularly to a non-emissive electrode for such tubes.

The broad object of our invention is to provide an electrode, such as a grid, from which primary and secondary emission is eliminated.

Another object is to provide an electrode of the character described which retains its non-emissive properties at high temperatures.

Still another object is to provide a tube embodying an electrode which will not become emissive by contamination with thorium from a thoriated filament.

The invention possesses other objects and features of advantage, some of which, with the foregoing, will be set forth in the following description of our invention. It is to be understood that we do not limit ourselves to this disclosure of species of our invention as we may adopt variant embodiments thereof within the scope of the claims.

Referring to the drawing, the figure is a perspective view of a tube embodying the improvements of our invention.

One of the most serious problems in vacuum tubes for transmission purposes is thermionic (primary) emission from the grid. Primary emission results in a reverse grid current which not only makes the tube unstable and erratic in its operation, but limits the output and prevents use of the tube in certain types of service. The problem is particularly aggravated in tubes where the grid normally runs at a relatively high temperature. Under these conditions usable grid materials are limited to refractory metals having high melting points, such as tungsten, tantalum, molybdenum and the like. These metals unfortunately are subject to contamination and exhibit undesirable amounts of primary emission.

There are two factors mainly responsive for primary grid emission. One is thermionic emission from the grid material per se, which depends upon the work function of the material used in making up the grid in the first instance. The other and most troublesome factor is lowering of the initial work function by contamination of the grid with material of higher emissivity such as thorium from a thoriated filament. Thus, even if a grid starts out as a non-emitter it ends up with high primary emission due to activation by thorium sputtered or otherwise deposited on it.

We have discovered an electrode material which exhibits substantially no primary emission,

2

even at high temperatures. Furthermore, the electrode does not become emissive by contamination with thorium. The improved electrode material is quite stable at high temperatures, and may be operated in elevated temperature regions where ordinary electrode materials would quickly fail.

Another feature of our improved electrode material is that it exhibits no secondary emission (electrons knocked out by impact). This absence of secondary electrons from an electrode is highly desirable in many cases.

In terms of broad inclusion, our improved non-emissive electrode comprises a metallic core having a stable surface layer including a refractory metal oxide. An alloy of refractory metals is preferably used for the core to facilitate formation of the desired surface composition. This electrode is enclosed in an evacuated envelope together with a thoriated cathode. While we have shown a tube embodying the improvements in the grid, it is understood that this is merely for purposes of illustration and that other electrodes may be rendered non-emissive in a like manner.

In greater detail, and referring to the drawing, the tube chosen to illustrate the invention comprises an envelope 2 of glass or the like having a reentrant stem 3 carrying an exhaust tubulation 4. A suitable base 6 having prongs 7 is cemented to the lower portions of the envelope. The triode illustrated contains a cathode 8, plate 9 and the improved grid 11, all coaxially disposed in the envelope. Plate 9 has a cap 12 connected by bracket 13 to a lead 14 sealed to the top of the envelope. The plate may be of any suitable material, such as molybdenum or tantalum, and, if desired, may be provided with a coating 15 of zirconium or the like to improve the gettering and heat radiating properties.

Cathode 8 is of the thoriated type, preferably a thoriated tungsten filament, comprising a coil welded at top and bottom to a pair of leads 17 sealed to stem 3. Flexible conductors 18 connect the cathode leads with a pair of base prongs. The thoriated cathode is preferred because our improved grid exhibits special non-emissive properties in such a combination. It is understood that the filament may assume other shapes than the spiral type illustrated.

Structurally speaking, grid 11 is preferably of the cage type comprising vertical wire bars terminating at a base ring 21 supported by bracket 22 on a pair of rods 23 sealed to stem 3. One of these rods functions as a lead and is connected

to a base prong by conductor 24. The shape of the grid and its mounting means may be varied within wide limits.

The improved grid is initially fabricated from an alloy of at least two refractory metals, preferably a tantalum-tungsten alloy comprising a major proportion of tantalum and a minor proportion of tungsten. A tantalum base alloy including about 93% tantalum and about 7% tungsten has given good results and is preferred. This alloy has a high melting point and sufficient ductility to permit fabrication of the grid structure. The alloy also has sufficient stiffness to provide a rigid grid capable of resisting shock and maintaining its position of alignment in the tube.

In order to improve the non-emitting properties of the grid we give it a special treatment. The first step is to oxidize the surface. This is preferably done by heating the grid in an oxidizing flame. Because the core includes tantalum and tungsten, oxides of both of these metals are formed on the surface. Furthermore, since the core is an alloy the oxides are thoroughly intermixed and exist in a finely divided state of subdivision. The degree and length of heating may be varied within wide limits, depending upon the depth of oxide layer desired.

The oxidized grid is preferably next heated in a reducing atmosphere such as hydrogen. The time and temperature of firing may be varied, satisfactory results being obtained by heating to around 1000° C. for about 3 minutes in an excess of hydrogen. The loss of weight involved points to at least a partial reduction of the tungsten oxide, this oxide either going to metal or to a lower order of oxide. Less reduction of the tantalum oxide is apt to occur because of the greater affinity of tantalum for oxygen. From the loss in weight measurements it is apparent that considerable oxygen is retained, hence the final composition includes the three elements: tantalum and tungsten and oxygen; the latter being combined as an oxide of at least one of these metals. It will be noted that one of the refractory metals has a greater affinity for oxygen than the other, resulting in a selective reduction. In other words, there is at least a partial reduction of the oxide of that metal having the lesser affinity for oxygen. Because the oxides initially formed from the alloy are in a very finely divided and intimately comingled state the resulting composition forms a dense, closely knit layer.

The appearance of the final coating is an enamel-like layer. It is probable that the metallic oxides or mixture of oxides and finely divided metal, by reason of their relative solubilities under the temperature conditions involved, combine to form a glass-like material of the nature of an intermetallic compound or a metalloid.

Stability of the surfacing layer is very important from the standpoint of tube life and where high temperature operation is involved. We have made a surfacing of tantalum oxide alone (formed by oxidizing a plain tantalum core) and found that our preferred surface layer exhibits non-emission properties for a materially longer time and under much higher temperatures.

Other combinations of refractory metals may be employed in the alloy core of the electrode. By the term "refractory metal" we mean metals in the class having a high melting point and relatively low vapor pressure, such as tungsten, tantalum and molybdenum. We have used a molyb-

denum-tungsten alloy with satisfactory results. In this case the oxides formed during the oxidation step are those of molybdenum and tungsten. During the reduction step some oxygen is lost, but there is not a complete reduction of both oxides. As in the example first described, the final coating composition includes at least two refractory metals and oxygen combined as an oxide of at least one of the metals. In both cases the core is surfaced with a layer composed of the partial reduction product from oxides of two refractory metals.

After the grid has been treated it is sealed into the envelope along with the plate and cathode; the latter being carbonized in accordance with the usual practice of making thoriated tungsten filaments. The tube to be exhausted is connected to a suitable vacuum pump through tubulation 4. During exhaust the electrodes are heated by suitable means, preferably by electron bombardment from the filament. This exhaust procedure is well understood by those skilled in the art. After exhaust the envelope is sealed off the pump and base 6 is applied.

If desired the step of firing the grid in hydrogen may be eliminated, and the heating of the grid in vacuum during exhaust of the tube relied upon to effect reduction. Heating the grid above about 1000° C. during evacuation accomplishes the desired purpose. Prefiring in a reducing atmosphere is preferred however as there is less chance of contaminating other electrodes in the tube.

The principle of operation underlying the improved grid is not fully understood. It is apparent however that the work function of the treated grid is increased so that the electrode material itself exhibits less primary emission at a given temperature. Its resistance to activation by thorium is less easily explained. The best theory seems to be that the surface layer maintains a reserve supply of oxygen for oxidizing thorium to its non-emissive oxide, thoria. The high stability of the surface layer on the grid has been pointed out, but this is not inconsistent with the theory because thorium has a tremendous affinity for oxygen. The tungsten component of the surface layer may enter into this by some catalytic action, in addition to performing the function of keeping the material stable at high temperatures by lowering its vapor pressure.

Whatever the correct explanation may be, we have conclusively demonstrated that the improved grid exhibits negligible primary and secondary emission and that the grid retains its non-emissive properties under high temperatures.

We claim:

1. A non-emissive electrode for electron tubes, said electrode having a surface layer consisting essentially of oxygen, tantalum and tungsten, the oxygen being combined as an oxide of at least one of said metals.

2. A non-emissive electrode having a surface layer consisting essentially of oxygen, tantalum and tungsten, the oxygen being combined as an oxide of tantalum.

3. An electron tube having a thoriated cathode and a non-emissive electrode, said electrode having a surface layer consisting essentially of tantalum and tungsten and oxygen combined as an oxide of at least one of said metals, for inhibiting primary emission on contamination of the electrode with thorium.

4. An electron tube having a thoriated cathode and a non-emissive electrode, said electrode hav-

ing a surface layer including in intimate admixture two refractory metals and oxygen combined as an oxide of at least one of said metals, for inhibiting primary emission on contamination of the electrode with thorium.

WILLIAM W. EITEL.

JACK A. McCULLOUGH.

## UNITED STATES PATENTS

| Number      | Name               | Date           |
|-------------|--------------------|----------------|
| 1,926,846   | Giard              | Sept. 12, 1933 |
| 1,871,363   | Fritz              | Aug. 9, 1932   |
| 5 1,558,961 | Bullimore          | Oct. 27, 1925  |
| 2,012,339   | Edwards et al.     | Aug. 27, 1935  |
| 2,238,596   | Mouromtseff et al. | Apr. 15, 1941  |
| 1,929,661   | Von Wedel          | Oct. 10, 1933  |

## REFERENCES CITED

The following references are of record in the 10 file of this patent: